

# UNITED STATES PATENT OFFICE.

GEORGE H. CAMPBELL, OF TORONTO, ONTARIO, CANADA.

## PROCESS OF PREPARING FLAX.

1,086,271.

No Drawing.

Specification of Letters Patent.

Patented Feb. 3, 1914.

Application filed March 11, 1910. Serial No. 548,700.

To all whom it may concern:

Be it known that I, GEORGE H. CAMPBELL, a citizen of Canada, and a resident of Toronto, in the county of York and Province 5 of Ontario, Canada, have invented certain new and useful Improvements in Processes of Preparing Flax, of which the following is a specification.

This invention relates to the preparation 10 of flax for the various purposes of the textile industry, and has in view a quicker and more economical treatment, and which will produce a greater yield than previously existing processes, all as now will be explained, 15 reference being had to the following specification and claims.

In carrying out this process, flax stalks or straw, in a dry state, are passed through a breaking machine, which removes the larger 20 portion of the various incrusting matters or shives, the diminution in weight of the straw treated being about forty-five (45) per cent. of the total original weight.

To render the stalks sufficiently dry, they 25 may be either air dried, or dried by the application of heat, the stalks being for this purpose placed on suitable shelves or frames, below which are placed pipes through which passes hot water or steam heated to a moderate 30 temperature.

After the stalks have been passed through the breaking machine, which may be of any ordinary and well-known kind, they will still contain a considerable proportion of 35 gummy, ligneous and other incrusting matters. For most uses the fiber requires further treatment to remove the larger portion or all of the shive material adhering to the fiber. This is done by a process of water 40 retting, which will now be described and which may be applied either immediately after the stalks come from the breaking machine, or after the fiber has been subjected to the various usual operations of scutching, 45 hackling, spinning, and weaving. In each of these various operations, tending to convert the broken stalks into yarn or cloth, the material progressively loses a certain amount of adhering incrusting material or 50 shives but not all. To remove the remainder the fiber is subjected to a process of retting. There are several methods of water retting, the process of water retting being here described in connection with the previous 55 operation of breaking.

By breaking the fiber before retting, the

water will act more quickly and thoroughly upon the gummy, ligneous, and other incrusting material attached to the fiber. The action of the water may be hastened by the 60 addition of certain chemicals or fermenting agents, or both, to the water used. The operation is then performed as in the ordinary process of water retting in which the unbroken stalks are immersed in the retting 65 water. By the preliminary removal of the larger portion of the shives the process of retting is not only hastened but the fiber produced is lighter in color than that obtained by the ordinary water retting process. 70 The action of the retting liquid may also be facilitated by keeping the flax or the liquid used in motion, which may be done by raising or lowering the flax in the containing vessel, or by blowing air through the liquid. 75 The air injected has also the advantage of assisting chemically in the process of retting or of fermentation, of putrefactive and other forms.

The water retting, with chemical, or ferments, or both, added to the retting water, although in many respects resembling chemical retting, is nevertheless practically distinguishable therefrom, by the small percentage of the ingredients added and by the 80 comparatively long time during which the process is carried on and principally by the fact that the main action is bacteriological.

Of the chemicals which may be added in very small proportions may be mentioned 90 the alkaline carbonates, bicarbonates and ammonia. The ferments added may be either in the form of retting liquor from a previous operation in a desired amount, or a ferment obtained by special culture. To 95 still further hasten and facilitate the fermentative or retting action, a food for the ferments may be added, such as cotton seed meal, linseed meal, bran or flour.

By the breaking of the dry stalks previous 100 to retting, the greater portion of the shives is eliminated at once, whereby the subsequent work to be done in the line of removal of shives or incrusting matter is diminished to that extent, and the subsequent step of 105 retting is very materially facilitated and shortened. Not only that, but the material will also be lighter in color than when ordinary water retting without previous breaking is used.

The fact that the retting period is shortened has also the advantage of a very consid-

erable increase in the yield of flax. In the ordinary process of water retting the yield of commercial flax is only about ten per cent. of the original weight of the stalks used, 5 while by this process the yield is increased up to fifteen per cent. or higher, even as high as twenty-five per cent. On account of the diminution in the time and quantity of putrefactive fermentation to which the 10 flax is subjected the fiber will suffer less diminution in tensile strength than by the old process of treatment.

After the retting is completed the material is dried at a low heat and subjected to 15 suitable mechanical manipulation to remove the loosened shive material. For this purpose the flax may be passed through a suitable breaking machine, preferably one having much finer grooves or teeth than were 20 used in the original breaking of the unretted flax stalks. In place of removing the shive material loosened through the operation of retting by passing the retted flax through 25 a breaking machine as stated, this loosened material may also be removed by means of scutching or beating machines, or by subjecting the flax to the action of other forms of machines, or to manual shive removing 30 operations.

The water retting here described, with or 35 without the addition of chemicals, ferment or foods, is preferably carried on at ordinary temperatures. Under the terms of ferment and food, are not included the small and adventitious quantities that may be found in the water or imperfectly cleaned containing vessels, but ferment, or food, or both, which has been separately added to the retting water in suitable proportions.

What I claim as new is:

1. In the art of preparing linen fibers, the improvement which consists in drying and breaking flax stalks, and retting the broken material in an aqueous solution having an 40 alkaline reaction.

2. In the art of preparing linen fibers, the improvement which consists in drying and breaking flax stalks, and retting the broken material in an aqueous liquid containing an added ferment.

3. In the art of preparing linen fibers, the improvement which consists in drying and breaking flax stalks, and retting the broken material in an alkaline solution containing an added ferment.

4. In the art of preparing linen fibers, the improvement which consists in drying and breaking flax stalks, and retting the broken material in aqueous solution containing an added ferment and an added food for the 60 ferment.

5. In the art of preparing linen fibers, the improvement which consists in drying and breaking flax stalks, and retting the broken material in an aqueous liquid and agitating 65 the material during the operation.

6. In the art of preparing linen fibers, the improvement which consists in drying and breaking flax stalks, and retting the broken material in an aqueous liquid and passing air through the liquid during the operation.

Signed at New York in the county of New York and State of N. Y., this 18th day of May, A. D. 1909.

GEORGE H. CAMPBELL.

Witnesses:

C. A. O. ROSELL,  
MABELLE A. DAVIS.